

# UNITED STATES PATENT OFFICE.

ARRIGO TEDESCO, OF TURIN, ITALY, ASSIGNOR TO SOCIETA ANONIMA STABILIMENTI BIAK, OF TURIN, ITALY, A COMPANY OF ITALY.

## ZINC ALLOY.

1,364,654.

Specification of Letters Patent.

Patented Jan. 4, 1921.

No Drawing.

Application filed April 11, 1919. Serial No. 289,388.

To all whom it may concern:

Be it known that I, ARRIGO TEDESCO, subject of the King of Italy, and resident of Turin, Italy, have invented certain new and 5 useful Improvements in Zinc Alloys, of which the following is a specification.

This invention has for its object a zinc alloy having a fine grained structure and being adapted both to be machined by means 10 of lathe, milling machine and generally by machine tools and to be worked by hot and cold forging and stamping, shearing, punching, holing and other metallurgical methods.

The alloy according to this invention is 15 chiefly formed of zinc which is the prevailing constituent thereof, with addition of iron, copper and manganese and one or more of following metals: cadmium, zirconium, nickel and aluminium.

20 The proportions of the various constituents may vary according to particular characters required from the alloy, the amount of said metals being comprised within the ranges stated by following table:

|    |              |         |       |          |
|----|--------------|---------|-------|----------|
| 25 | Zinc-----    | from 85 | to 96 | percent. |
|    | Cadmium ---  | " 0,3   | " 0,7 | "        |
|    | Nickel ----- | " 0,5   | " 8,0 | "        |
|    | Iron-----    | " 0,5   | " 1,9 | "        |
|    | Aluminium--- | " 2,5   | " 7,1 | "        |
| 30 | Zirconium--- | " 1,2   | " 2,5 | "        |
|    | Manganese--- | " 0,3   | " 0,9 | "        |
|    | Copper ----- | " 2,0   | " 8,0 | "        |

One or more among cadmium, zirconium, nickel and aluminium may be omitted in the alloy but at least one of them must be contained.

It has been found that satisfactory results are obtained by using a large proportion of nickel that is up to 8 per cent. as above stated; by way of example an alloy of this 40 class containing 4 per cent. of nickel shows a resistance to tensile strength of about 24 kg. per square mm.

In any case the alloy according to this invention, while having a reduced cost owing 45 to the large percentage of zinc contained therein, is provided, because of additions above referred to, with a satisfactory resistance both to mechanical stresses and chemical actions and with a fine grained structure 50 causing it to be adapted to any kind of machining and working methods.

What I claim as my invention and desire to secure by United States Letters Patent is:

A zinc alloy, comprising zinc in proportion exceeding 85%, copper in proportion between 2 and 8%, aluminum in proportion between 2.5 and 7.1%, and nickel in proportion between 0.5 and 8%, together with a small addition of iron and manganese. 55 60

Signed at Turin, Italy, this 13th day of March, A. D. 1919.

ARRIGO TEDESCO.